

June 15, 1926.

1,589,325

S. E. SHEPPARD ET AL

ELECTRODEPOSITING ORGANIC MATERIAL SUCH AS RUBBER UPON  
POROUS OBJECTS OF NONCONDUCTING MATERIAL SUCH AS FABRICS  
Filed April 1, 1926



INVENTORS,  
*Samuel E. Sheppard & Carl L. Beal,*  
BY *P. L. Stinchfield*  
ATTORNEY.

Patented June 15, 1926.

## UNITED STATES PATENT OFFICE.

SAMUEL E. SHEPPARD AND CARL L. BEAL, OF ROCHESTER, NEW YORK, ASSIGNEES TO  
EASTMAN KODAK COMPANY, OF ROCHESTER, NEW YORK, A CORPORATION OF  
NEW YORK.

ELECTRODEPOSITING ORGANIC MATERIAL SUCH AS RUBBER UPON POROUS OBJECTS  
OF NONCONDUCTING MATERIAL SUCH AS FABRICS.

Application filed April 1, 1926. Serial No. 99,079.

This invention relates to processes of electrodepositing organic material, such as rubber, upon porous objects of non-conducting material, such as fabrics. One object 5 of the invention is to provide a process of this character in which the electrodeposition will be very accurately controlled. Another object of the invention is to provide such a process in which evenness of the deposit is insured. Still another object of the invention is to provide such a process in which certain steps predetermine the degree of penetration of the deposit into the porous material or fabric. Another object of 10 the invention is to provide good adhesion between the deposited substance and the material on which it is deposited. Other objects will hereinafter appear.

In the accompanying drawing the single 20 figure is a diagrammatic sectional view of one form of apparatus in which our process may be carried out, the relative sizes of the parts being exaggerated for the sake of clearness.

25 In U. S. Patent No. 1,476,374, Sheppard and Eberlin, December 4th, 1923, for electrodeposition of rubber coatings it is stated that the electrodeposition of rubber from emulsions thereof can be carried out upon 30 porous non-conducting objects, such as wood, for example, by impregnating them with solutions of electrolytes. This principle is of general applicability to all porous objects of non-conducting materials, 35 such as cloth and similar fabrics. A continuous method of electrodepositing organic materials from aqueous emulsions thereof onto fabrics is disclosed in copending application Serial No. 35,612, Sheppard and 40 Eberlin, filed June 8th, 1925, for electrodeposition of rubber under gas-removing conditions.

In the deposition of the minute particles 45 of organic material, such as rubber, upon the fabric or other porous material, it is desirable to control the depth of penetration of the deposit into the pores. For example, it may be desirable to provide a deposit all the way through the fabric so as 50 to thoroughly impregnate it with the coating substance, such as rubber. On the other hand it may be desirable at times to confine the deposit practically to one surface of the fabric. For the production of certain water-proofed cloths the impregnation 55 may be intermediate between the two extremes indicated above. Moreover, it may be useful to lightly waterproof the threads or fibers of the fabric by effecting a light 60 deposit upon them.

We have found that the depth and character of the deposit can be controlled by adding a size containing a coagulant to the porous object of non-conducting material, such as the fabric, before the electrodeposition takes place. In general we prefer to use acid hydrophilous colloids which are typified by such substances as glue, starch, dextrin, etc. In the preferred form of our 65 invention we use such colloids having a pH 70 value greater than 3 and less than 7. Of course, the depth to which the size is forced into the fabric adds a feature of control in addition to the acid or coagulant mentioned above.

75 It is also highly desirable to provide uniform deposits. Even where the size mentioned above is uniformly associated with the fabric, or other porous object, unevenness may occur through the uneven wetting 80 ability of fibers in different parts of the fabric. This is due to the presence of anti-wetting substances, such as grease, oil and the like. We have found it desirable, where such deleterious substances are present, to 85 subject the fabric, or other porous object, to a treatment which removes the anti-wetting substances, such treatment comprising in the preferred form of our invention an immersion in an alkaline degreasing bath.

90 We shall now describe the preferred embodiment of our invention by way of illustration, but it will be understood that our invention is not limited to the details thus given, except as indicated in the appended 95 claims.

Referring to the accompanying drawing, the porous non-conducting material, say a cotton cloth, such as is commonly used for the preparation of waterproof rubberized sheets, is unwound from roll 1 and 100 passed through a bath 2 for removing anti-wetting substances. It may be conveniently led beneath a roll 3 which keeps it properly immersed. At the top of the tank are guide and squeezing rolls 4. In the tank any suitable bath may be employed. We have found 105

- that an alkaline degreasing bath is particularly effective, such as a 5% aqueous solution of sodium sulfite. Of the great many useful alkalies that may be employed, we note also 5 sodium carbonate, tri-sodium phosphate and sodium bisulfite. The excess of degreasing solution is squeezed out of the fabric by the rolls 4 and the fabric then passes through tanks 5 and 6 in which it is washed by water.
- 10 Between each tank and the next are located additional guide and squeeze rolls 7 and 8. After having been freed from anti-wetting substances and having been thoroughly washed, the cloth next passes into the bath 15 of size 9. It may be held below the solution by a lower roll 3, similar to the rolls in the previous tanks. The cloth then passes up between the guide and squeeze rolls 10 and over the further guide roll 11.
- 20 For a heavy proofing on thin fabrics we prefer to use a somewhat viscous size such as a 10 to 15% starch solution at 160 to 180° F., or a 5 to 10% glue solution, or a .5 to 1% solution of agar-agar. The sizing material 25 enters into the pores or openings in the fabric, or other porous non-conducting material, and improves the smoothness of the coating which is electrodeposited. These sizes may be varied in acidity from almost 30 neutral to say pH3, the most useful range being pH values greater than 3 and less than 7. The acids which we prefer to employ are the inexpensive and easily controlled organic ones, such as acetic, formic, 35 oxalic or lactic. The initial acidity of the size assists greatly the "striking" or initial deposit of the particles from the emulsion upon the fibers and in the pores of the fabric. This is probably due to a slight coagulating effect. Moreover, the acidity of the 40 size has the further advantage of preventing the rubber particles from passing entirely through the fabric and onto the metal anode, which will be hereinafter described.
- 45 Where only a light proofing is required, less concentrated and less viscous sizes than those just described above may be employed. They will be varied also with the closeness of texture and thickness of the fabric, as will 50 be understood by those skilled in the art.
- Where it is desirable to impregnate the fabric with the deposit only slightly on one side of it, a slightly acid and rather viscous size is used, say one having a pH value of 5 to 4.
- 55 The fabric is thoroughly impregnated with this size and then electrodeposition carried on as hereinafter described. Besides controlling the degree of penetration of the coating a firm adhesion of the deposit to the fabric 60 can be obtained.
- Sometimes it is desirable to have the deposit extend thoroughly through the fabric and on both faces thereof. In this case we use a size, the acidity of which is very slight 65 or almost neutral, say one having a pH value under 7 but above 5. This size is not worked into the fabric but is merely applied to the back of it (the side opposite the one from which the electrodeposited particles come). This application is preferably made just 70 prior to the electrodeposition process, so that there will be little, if any, chance for the size to soak into the fabric. The mechanical expedients for coating one face of a fabric with a viscous material, such as a size, are 75 well known and need not be described further.
- For very light waterproofing or "shower-proofing", rubber may be electrodeposited after a special adjustment of the size. The 80 fabric is coated on the back with a thin size such, for example, as an aqueous solution containing from .1 to .3% agar-agar and about .2% acetic acid. We have likewise found it useful to modify the bath by 85 adding a small amount of a buffering electrolyte, such as sodium sulfite,—say .3 to .5%. With this sizing, properly applied, as specified above, there is obtained, upon electrodeposition, a soft even deposit which, 90 when dry, covers all the threads with a thin clear rubber coating, completely waterproofing the cloth without hiding its weave.
- The acidification of the size baths may be modified or controlled by the addition of 95 other electrolytes, such as acid salts, highly ionized neutral salts, or even non-electrolytes, such as alcohol, which have a coagulating action upon the emulsion of rubber or other organic material. 100
- The properly sized fabric next passes over the surface of an anode in the electroplating bath of rubber emulsion, the latter being indicated at 12 in the drawing. For such anode we prefer a rotary metallic 105 drum 13. Suitable cooperating cathodes are shown at 14. In any event the sized fabric passes adjacent the anode in the path of the current.
- The bath from which the organic material is electrodeposited may be an aqueous emulsion of the kind disclosed in the above cited Patent No. 1,476,374 or the one described in the application of Sheppard and Eberlin, Serial No. 21,340, filed April 7th, 110 1925, for aqueous emulsion of unvulcanized rubber and sulfur. Other useful baths are disclosed, for instance, in application Serial No. 21,342 Eberlin and Beal, filed April 7th, 115 1925, for aqueous emulsions of electrodepositable cellulosic compounds and coalescing agents therefor and in application Serial No. 25,160 Sheppard and Beal, filed April 22nd, 1925, for electrodeposition of organic materials such as rubber and cellulosic compounds. The above mentioned baths are, of course, merely typical ones and any suitable aqueous emulsion containing organic material in the electrodepositable state may be used in connection with 120 125 130

the proper kind of porous object or fabric. See also application Serial No. 611,162 Shepard and Eberlin, filed January 6th, 1923.

It will be noted that all of these baths 5 contain not only the primary organic coating material but substances which assist the formation or perfection of the coating. For example, the deposition of the rubber includes the simultaneous passage of sulfur 10 and other conditioning agents, such as accelerators and pigments into the deposit. This permits the rubber to be vulcanized in the exact place where it is deposited in the porous object or fabric. Hereinafter when 15 aqueous emulsions of rubber or organic coating materials are referred to, it will be understood that these terms include not only aqueous emulsions of rubber or such materials by themselves, but likewise and 20 preferably emulsions in which the rubber or organic material is associated with one or more conditioning agents which pass with it into the deposit.

Having thus described our invention, 25 what we claim as new and desire to secure by Letters Patent is:

1. The process of electrodepositing organic coating material upon porous objects of non-conducting material which comprises 30 the steps of adding to said objects a size containing a coagulant and bringing said sized object into contact with an aqueous electro-conducting emulsion of said organic coating material and passing an electrodepositing current through said emulsion with said object adjacent the anode in the 35 path of the current.

2. The process of electrodepositing organic coating material upon porous objects 40 of non-conducting material which comprises the steps of removing anti-wetting substances from an object until it is substantially uniformly wettable, adding to said object a size containing a coagulant, bringing said sized object into contact with an aqueous electroconducting emulsion of said organic coating material, and passing an electrodepositing current through said emulsion with said object adjacent the anode 45 in the path of the current.

3. The process of electrodepositing organic coating material upon porous objects of non-conducting material which comprises the steps of treating an object with 50 an alkaline degreasing compound, thereafter associating with said object a size containing a coagulant, bringing said sized object into contact with an aqueous electroconducting emulsion of said organic coating material and passing an electrodepositing current through said emulsion and object.

4. The process of electrodepositing organic 55 coating material upon porous objects of non-conducting material which comprises the

steps of associating with an object a size comprising acid hydrophilous colloid, bringing said sized object into contact with an aqueous electroconducting emulsion of said organic coating material and passing an electrodepositing current through said emulsion with the said object in position to receive the resulting deposit. 70

5. The process of electrodepositing organic coating material upon porous objects of 75 non-conducting material which comprises the steps of removing anti-wetting substances from an object until the latter is substantially uniformly wettable, associating with said object a size comprising an acid hydrophilous colloid, bringing said sized object into contact with an aqueous electroconducting emulsion of said organic coating material, and passing an electrodepositing current through said emulsion with said object in the path of the current to receive a 80 deposit. 85

6. The process of electrodepositing rubber upon porous objects of non-conducting material which comprises the steps of associating 90 with an object a size containing an acid hydrophilous colloid, bringing said object into contact with an aqueous electroconducting rubber emulsion, and passing an electrodepositing current through said emulsion with said object adjacent the anode in the 95 path of the current.

7. The process of electrodepositing rubber upon fabrics of non-conducting material 100 which comprises associating with said fabric a size containing a hydrophilous colloid having a pH value greater than 3 and less than 7, bringing said sized fabric into contact with an aqueous electroconducting emulsion of rubber and passing an electrodepositing current through said emulsion with said fabric in a position to receive the resulting deposit. 105

8. The process of electrodepositing rubber upon fabrics of non-conducting material 110 which comprises, removing anti-wetting substances from the fabric until it is substantially uniformly wettable, associating therewith a size containing a hydrophilous colloid having a pH value greater than 3 and less than 7, and bringing said sized fabric into contact with an aqueous electroconducting emulsion of rubber and passing an electrodepositing current through said emulsion with said fabric adjacent the anode in the 115 path of the current. 120

9. The process of electrodepositing rubber upon fabrics of non-conducting material 125 which comprises adding to said fabrics a size containing a hydrophilous colloid having a pH value greater than 3 and less than 7, and bringing said sized fabric into contact with an aqueous electroconducting emulsion of rubber and passing an electrodepositing current through said emulsion 130

- with said fabric adjacent the anode in the path of the current, the extent to which the size enters the fabric and the acidity of the size being adjusted to control the penetration and character of the deposit.
10. The process of electrodepositing rubber upon cloth which comprises treating the cloth with an alkaline degreasing liquid, freeing it from said degreasing liquid, associating with it a sizing comprising a hydrophilous colloid having a pH value greater than 3 and less than 7, bringing said sized cloth into an aqueous electroconducting emulsion of rubber and passing an electrodepositing current through said emulsion with said current adjacent the anode in the path of the current.
15. Signed at Rochester, New York, this 26th day of March, 1926.

SAMUEL E. SHEPPARD.  
CARL L. BEAL.